

## UNITED STATES PATENT OFFICE

JOHN SCHUBER, OF ASHEVILLE, NORTH CAROLINA, ASSIGNOR TO THE CHAMPION FIBRE COMPANY, OF CANTON, NORTH CAROLINA, A CORPORATION OF OHIO

## BLEACHING CELLULOSE PULP

No Drawing.

Application filed June 30, 1928. Serial No. 289,636.

This invention relates to a process of bleaching cellulose pulp involving the use of an oxidizing bleaching agent, and is particularly concerned with such a process adapted to produce from raw chemical pulp, 5 particularly, raw sulfate or sulfite pulp,—a bleached pulp capable of yielding a paper product possessing not only a high degree of relative whiteness (i. e., "high color") but 10 also a high degree of resistance to fold and to tear.

In the bleaching of cellulose pulp a high color is obtained generally only at the sacrifice in the final paper making product either 15 of strength, of yield, or of resistance to fold and to tear, or of all of these. For example, it is known that the alpha, or resistant, cellulose content of sulfite pulp may be increased to a value well over 90% by treatment 20 with hot caustic alkali in connection with the bleaching process. While the paper product from the bleached pulp thus obtained possesses a high degree both of relative whiteness and of resistance to fold and 25 to tear, the process results in a highly disadvantageous material loss of the raw pulp substance; in addition, this procedure is open to the objections that it is time consuming and requires large amounts of caustic alkali 30 and of steam. Also, it has been attempted to improve the color of kraft or sulfate pulp by treating the same with a solution containing a sulfite or bisulfite prior to the bleaching treatment with an oxidizing bleaching agent. 35 This procedure, it has been found, is time consuming and fails in effecting a relative whiteness, strength, or softness in the final paper product obtained from this bleached kraft pulp comparable with the whiteness, 40 strength, or softness of papers produced from ordinary commercial grades of bleached sulfate pulp.

An object of the present invention, therefore, is to provide an economical process of 45 bleaching raw cellulose pulp whereby to ef-

fect the production of a bleached pulp not only possessing a high degree of relative whiteness but also capable of yielding a final paper product having a desirable resistance to fold and to tear. Another object is to provide such a process whereby to conserve the maximum amount of pulp substance.

I have found that the above and other desiderata may be effected by: first, subjecting unbleached or raw cellulose pulp in aqueous suspension to a mild bleaching treatment with an oxidizing bleaching agent; second, adding to the so-treated pulp a suitable acid reducing agent in an amount sufficient to bring the pulp suspension to an acidity represented by a pH value of from 4.0 to 2.0; 60 third, removing soluble residues from the pulp suspension by thorough washing; and fourth, treating the thoroughly washed pulp in aqueous suspension with an oxidizing bleaching agent in such proportions as to produce the desired relative whiteness of the pulp. A final washing operation, with water, may, of course, be carried out. Or, the bleached pulp,—after being treated in accordance with operations one to four inclusive as above set out,—may be subjected to the action of an acid reducing agent, followed by a thorough washing with water. By "a mild treatment" with an oxidizing 65 bleaching agent I mean a treatment carried out under such conditions, including proportion of bleaching agent to pulp, as not materially to impair the strength of the final product. 70

The use of an acid reducing agent, between stages of bleaching with an oxidizing bleaching agent, under such conditions as to give a degree of acidity of the pulp suspension represented by pH values of from 4.0 to 2.0, 75 greatly aids in the removal by water washing of those compounds and materials in the partially bleached pulp which, if not removed, interfere with or negative the efficacy of a subsequent treatment with the oxidizing 80 agent.

bleaching agent. If the pH value of the pulp is greater than 4.0, the degree of acidity is so low that the detrimental materials are not thoroughly removed; if, on the other hand, the pH value of the pulp is less than 2.0, the degree of acidity is so high that the strength of the fiber may be impaired and the desired results therefore lost.

While the invention is not limited to the use of any specific acid reducing agent,—it being essential only that the acid reducing agent be of such a character that it may be added to the pulp suspension in such an amount as to give thereto an acidity represented by a pH value of from 4.0 to 2.0,—I prefer to employ an aqueous solution of sulfur dioxide. However, any other suitable acid reducing agent, such as, for example a solution containing stannous chloride and hydrochloric acid may be used.

It is common knowledge that, when unbleached chemical pulp is subjected to the action of an oxidizing bleaching agent,—e. g., bleaching powder,—in increasing proportions, there is a critical proportion of bleach to fiber beyond which the action of the bleach results in a loss of fiber strength without materially increasing the whiteness. This critical point depends to some extent upon the varying factors of the pulping process by which the pulp is produced.

In the process according to the present invention there is used in the first stage of bleaching an amount of oxidizing bleaching agent which is known to be less than the critical amount but sufficient to cause a material bleaching effect.

The soluble products associated with the pulp after this first stage of bleaching may be removed therefrom prior to the addition of the acid reducing agent; this is not essential, and in fact there results a greater economy in those cases where the acid reducing agent is added to the partially bleached pulp before the washing operation. Thorough washing of the pulp after treatment with the acid reducing agent is essential to the successful operation of the process. The removal by washing of appreciable quantities of colloidal coloring matter makes it possible to complete the bleaching with a marked reduction in consumption of bleach, and removal of coloring materials not easily attackable by the bleach makes it possible, without material loss of strength of the pulp, to continue the bleaching until the color of the pulp, in the case of soda and sulfate or kraft pulp, is comparable with that of commercial bleached sulfite, and is superior to that of the usual commercial sulfite in the case of sulfite pulp.

The length of time during which the acid reducing agent reacts with pulp is an important element in the successful operation of the process. While I have observed favorable results after one minute of reaction, more

favorable results are obtained as the time of reaction is increased up to thirty to forty-five minutes.

The acid reducing agent when present in the above stated amount apparently has the property of reducing the positive electric charges upon (1) certain agents,—probably mineral catalytic agents,—normally present in the pulp, which agents when allowed to remain in the pulp during the bleaching treatment with the oxidizing bleaching agent result in the destruction of the strength of the fiber, and (2) the colloidal organic matter which is present as a by-product of the primary bleaching treatment. Were these agents and by-products allowed to remain in the pulp during the entire period of bleaching, excessive proportions of bleach would be consumed without the production of a high degree of relative whiteness; such excessive proportions of bleach cause a material reduction in the strength value of the resulting bleached pulp. Reducing the positive electric charges upon the said agents and the said by-products makes it possible easily to remove these materials by water washing. Addition of the acid reducing agent prior to bleaching provides for the removal of at least a part of the "catalysts" detrimental to the strength of the pulp but does not provide for the removal of the by-products of bleaching, while the addition of acid reducing agent after the bleaching treatment has been concluded does provide for the removal either of "catalysts" or of by-products only after the same have exerted their detrimental effect upon the whiteness and/or strength of the finished pulp.

Whatever may be the correct explanation of the mechanics of my process it is a fact that by it there may be produced from pulps obtained by any of the several chemical pulping processes, bleached pulps which are more nearly white than are the hitherto known bleached pulps, without material loss in substance, and without material loss in strength, or in resistance to fold and to tear, of the final paper product.

As illustrating in greater detail in what manner the process according to the present invention may be carried out in connection with the bleaching of sulfate pulp produced from pine wood, the characteristics of which pulp depend more or less upon the varying factors of the pulping process by which it is produced, it may be assumed, for example, that the unbleached sulfate pulp has a maximum ball mill bursting strength of 142 points per pound per ream of  $24 \times 36''$ —480, and a tear at maximum bursting strength of 3.67 grams per pound per ream. A 10% stock suspension of this unbleached sulfate pulp is treated with a solution of bleaching powder in amount equal to 14% based upon the weights of the dry pulp substance and of

the calcium hypochlorite powder containing 35% available chlorine, or 62.5% of the total bleach used in both stages of bleaching. When the available chlorine has become exhausted or nearly so the pulp, together with the by-products of bleaching, is treated, without or with an intervening washing operation, with a solution of sulfur dioxide in an amount sufficient to bring the pulp suspension to an acidity represented by a pH value of from 4.0 to 2.0. I have found that a pH value of about 3.2 gives the best and most economical results. For that purpose there is required approximately 1% of sulfur dioxide based on the dry weight of the pulp.

Sufficient water is added to the reaction mass to produce a stock suspension of approximately 3%, which suspension is agitated for from 30 to 45 minutes and thereafter is thoroughly washed with water to the removal of all soluble matter. A 3% stock suspension of the resulting washed pulp is then bleached with 8.4% of bleaching powder, and washed. The final washed product is characterized by a bursting strength of 137 points per pound per ream, a tearing strength of 3.15 grams per pound per ream, a folding endurance of 43 double folds per pound per ream, an alpha (or resistant) cellulose content (determined on the pulp) of 84.6%, and a degree of relative whiteness comparable with that of commercial bleached sulfite pulp. The pulp product may be brought to a still higher degree of relative whiteness by preceding the final washing by a treatment with an acid reducing agent such as that hereinbefore described.

A product made from the same unbleached sulfate pulp treated as in the manner above described except that the treatment with sulfur dioxide was omitted and that the second stage of bleaching was effected with 13% of bleaching powder (rather than 8.4%) was characterized by a bursting strength of 115 points per pound per ream, a tearing strength of 2.67 grams per pound per ream, a folding endurance of 22 double folds per pound per ream, an alpha (or resistant) cellulose content (determined on the pulp) of from 78 to 81%, and a color which was far below that of ordinary commercial sulfite pulp.

While in the above example I have indicated certain specific values and have stated certain specific proportions of the several reagents, I would not consider it to be a departure from the scope of this invention to change these proportions within the broad limits hereinbefore mentioned, or to substitute for sulfur dioxide,—the specific acid reducing agent of the example,—another acid reducing agent capable of imparting to the pulp suspension an acidity represented by a pH value of from 4.0 to 2.0. It is to be understood, also, that the invention herein described and hereinafter claimed may success-

fully be practiced with the use of any known oxidizing bleaching agent, and that by the expression "a hypochlorite bleaching agent" in certain of the appended claims I mean to include also known equivalents thereof.

I claim:

1. Process for treating a cellulose pulp to produce therefrom a paper making product of high color and a high degree of resistance to fold and to tear which comprises subjecting the pulp to a mild bleaching treatment with an oxidizing bleaching agent, adding to the resulting partially bleached pulp in aqueous suspension an acid reducing agent in an amount sufficient to impart thereto an acidity represented by a pH value of from 4.0 to 2.0, thoroughly washing the so treated pulp, and thereafter bleaching the washed pulp with an additional amount of an oxidizing bleaching agent.

2. Process for treating a cellulose pulp to produce therefrom a paper making product of high color and a high degree of resistance to fold and to tear which comprises subjecting the pulp to a mild bleaching treatment with a hypochlorite bleaching agent, adding to the resulting partially bleached pulp in aqueous suspension an acid reducing agent in an amount sufficient to impart thereto an acidity represented by a pH value of from 4.0 to 2.0, thoroughly washing the so treated pulp, and thereafter bleaching the washed pulp with an additional amount of a hypochlorite bleaching agent.

3. Process for treating a cellulose pulp to produce therefrom a paper making product of high color and a high degree of resistance to fold and to tear which comprises subjecting the pulp to a mild bleaching treatment with an oxidizing bleaching agent, adding to the resulting partially bleached pulp in aqueous suspension a solution of sulfur dioxide in an amount sufficient to impart thereto an acidity represented by a pH value of from 4.0 to 2.0, thoroughly washing the so treated pulp, and thereafter bleaching the washed pulp with an additional amount of an oxidizing bleaching agent.

4. Process for treating a cellulose pulp to produce therefrom a paper making product of high color and a high degree of resistance to fold and to tear which comprises subjecting the pulp to a mild bleaching treatment with an oxidizing bleaching agent, adding to the resulting partially bleached pulp in aqueous suspension an acid reducing agent in an amount sufficient to impart thereto an acidity represented by a pH value of from 4.0 to 2.0, thoroughly washing the so treated pulp, thereafter bleaching the washed pulp with an additional amount of oxidizing bleaching agent, treating the bleached pulp with an acid reducing agent in amount sufficient to impart thereto an acidity repre-

sented by a pH value of from 4.0 to 2.0, and finally thoroughly washing the so treated pulp.

5. Process of bleaching cellulose pulp by means of an oxidizing bleaching agent in one or more stages characterized by a treatment of the pulp after one of said stages in aqueous suspension with an acid reducing agent in amount sufficient to impart to the pulp suspension an acidity represented by a pH value of from 4.0 to 2.0.

6. Process of bleaching cellulose pulp as defined in claim 5, in which the treatment with acid reducing agent follows a mild treatment with an oxidizing bleaching agent.

15 In testimony whereof, I affix my signature.

JOHN SCHUBER.

20

25

30

50

55